

## 1

2,923,627

## COLOUR PHOTOGRAPHY

Leslie Frederick Alfred Mason, Ilford, England, assignor to Ilford Limited, Ilford, England, a British company

No Drawing. Application March 31, 1958  
Serial No. 724,931

Claims priority, application Great Britain April 17, 1957

## 11 Claims. (Cl. 96—56)

This invention relates to colour photography and more particularly to developing compositions for use in colour photographic processes.

In one well-known method of colour photography a colour image is formed by developing a silver salt image in a photographic element by means of a developing solution which contains an aromatic primary amino developing agent and a dye intermediate (hereinafter referred to as a colour coupler) such that the oxidation products of the developing agent formed during its developing action couple with the colour coupler to constitute a dye in situ with the developed silver image, the dye commonly being an azomethine or quinone-imine dye.

The developing agents used in this type of process are usually derivatives of p-phenylene diamine, well-known examples being N,N-diethyl p-phenylene diamine and 2-amino-5-diethyl amino toluene and their salts and sulphur dioxide reaction products. These agents unfortunately have a tendency to oxidise in the air and, since the oxidation products will combine with the colour coupler present, the solutions in use acquire, more or less rapidly, a scum consisting mainly of the dye thus formed. This is so serious a difficulty that such developers must frequently be discarded long before they have outlived their useful activity.

The extent of scum formation depends on the extent of aerial oxidation which occurs, and this in turn is found to be greatest at higher pH values. Accordingly, a balance must be struck between the activity of the developer, which is reduced by lowering the pH of the solution, and the liability of the developer to oxidation, which is increased by increasing the pH of the solution, i.e. some sacrifice of developer activity must be made in order to avoid undue oxidation. Generally, the pH of the solutions is adjusted to about 10.5.

In an effort to overcome this difficulty, various anti-oxidants have been described for inclusion in the developer, probably the best known being ascorbic acid. However, the inclusion of such anti-oxidants generally causes some loss in developer activity. Moreover, only very small quantities must be used so that the addition of the precise quantity required in any particular case is a highly critical operation. Moreover, they generally only hold the solution against scum formation for a matter of 2 to 3 hours.

It has been proposed to include hydroxylamine or a salt thereof in colour developers as an anti-oxidant or preservative. However, on attempting to use this additive for a colour developer containing colour coupler, at the usual pH value of about 10.5, it was found that it failed entirely of its purpose, i.e. it had little or no effect on the formation of dye scum.

It has been found, however, that if the pH of the developing solution containing a colour coupler is increased, so that the tendency to form dye scum is enhanced, the addition of hydroxylamine or a salt thereof becomes effective in reducing, or even eliminating, dye scum. It

## 2

will be appreciated that this result is highly surprising since an increase in pH would have been expected to make the position worse rather than better.

Thus, a photographic developing composition for use in colour developing a developable silver salt image in a photographic element may comprise an aromatic primary amino developing agent, a colour coupler which is capable of combining with the oxidation products of such developer to form a dye, and hydroxylamine or a salt thereof, the said composition on dissolution in water having a pH of at least 11.25.

Whilst developers thus formulated are of very considerable value it is, as noted above, based on the possibility of using developing solutions at pH values of at least 11.25. In some developing steps, however, such high pH values are not practicable since they lead to other difficulties.

In British Patent No. 782,304 it is explained that resistance to aerial oxidation in developers of the character referred to above can also be obtained by the inclusion in the developer of a small quantity of a 4-aryl-2-oxytetronic acid or 4-aryl-2-oxytetronimide. These compounds may be written in tautomeric form as follows:



30 where R is an aryl group or a substituted aryl group and X is an oxygen atom or animino group. The aryl group R may be a phenyl or naphthyl group or a corresponding group containing, for example, alkyl, aralkyl, aryl, sulphonic acid or halogen substituents. Specific compounds of value are:

35 4-phenyl-2-oxytetronimide  
4-0-sulphophenyl-2-oxytetronimide  
4-0-chlorophenyl-2-oxytetronimide  
4-0-chlorophenyl-2-oxytetronic acid

40 In practice these compounds delay the onset of scum formation for a period of the order of 4 hours.

It has now been discovered that, surprisingly, hydroxylamine and either ascorbic acid or a compound of the formula given above exert a synergistic effect, even at the 45 pH values ordinarily used for colour developers, i.e. 9 to 11.25, so that while hydroxylamine is inactive when used alone and the others are effective to delay scum formation by only about 4 hours at most, the combination delays scum formation for periods of the order of 12 hours, or even substantially longer.

50 According to the present invention therefore a photographic developing composition for use in colour developing a developable silver salt image in a photographic element comprises an aqueous alkaline solution of an aromatic primary amino developing agent, a colour coupler which is capable of combining with the oxidation products of such developer to form a dye, hydroxylamine or a salt thereof and ascorbic acid and/or a tetronic compound of the formula above set forth. The invention further includes processes of colour development employing such solutions.

55 It is to be understood that the specific description of the production of the tetronic compounds is to be found in British Patent No. 782,304.

60 The proportions of hydroxylamine and ascorbic acid or tetronic compound are not unduly critical. Generally a quantity of the order of 0.5 to 1.5 g./litre of hydroxylamine is suitable and proportions of 0.1 to 0.5 g./litre of ascorbic acid or tetronic compound, or mixture of these.

65 Preferably according to the invention the developing agents are N,N-diethyl p-phenylene diamine or 2-amino-5-diethyl amino toluene, or their salts or sulphur dioxide

reaction products. A suitable alkalinity in the developing composition is conveniently achieved by the use of alkali carbonates or, where a high pH is desired, mixtures of tribasic sodium phosphate and dibasic sodium phosphate, these latter compounds being particularly useful owing to their good buffering properties.

It will be appreciated that the developing compositions of the invention may include other ingredients common to photographic developers, e.g. alkali, ammonium or amine sulphites and alkali or ammonium bromides. It is also frequently of advantage to include a proportion of ethyl alcohol in the developer.

Where the developing compositions are formulated and marketed rather than being used directly, it is generally desirable that the colour coupler and the alkali should be packed separately from the developing agent, hydroxylamine and ascorbic acid or tetronic compound as referred to above. The invention accordingly further includes in solid form or in strong aqueous solution a composition of aromatic primary amino developing agent, hydroxylamine and ascorbic acid and/or tetronic compound as defined.

The following examples, in which the developers identified as developers D, E, F, G and H are in accordance with the invention, will serve to illustrate the invention:

#### Examples

| Developer formulations                           | A         | B         | C         | D         | E         | F         | G         |
|--------------------------------------------------|-----------|-----------|-----------|-----------|-----------|-----------|-----------|
| Sodium carbonate (10 H <sub>2</sub> O)           | g. 80     | g. 80     | g. 80     | g. 80     | g. 80     | g. 80     | g. 80     |
| Sodium hexametaphosphate                         | g. 3      | g. 3      | g. 3      | g. 3      | g. 3      | g. 3      | g. 3      |
| Hydroxylamine hydrochloride                      | g. 1      | —         | —         | g. 1      | g. 1      | g. 1      | g. 1      |
| Ascorbic acid                                    | g. 0.2    | —         | —         | g. 0.2    | —         | —         | —         |
| 4-o-sulphophenyl-2-oxytetronimide                | g. —      | —         | —         | g. —      | —         | —         | —         |
| 4-o-chlorophenyl-2-oxytetronimide                | g. —      | —         | —         | g. —      | —         | —         | —         |
| 4-phenyl-2-oxytetronimide                        | g. —      | —         | —         | —         | —         | —         | g. 0.2    |
| Sodium sulphite                                  | g. 5      | g. 5      | g. 5      | g. 5      | g. 5      | g. 5      | g. 5      |
| Potassium bromide                                | g. 2      | g. 2      | g. 2      | g. 2      | g. 2      | g. 2      | g. 2      |
| Industrial spirit 74° O.P.                       | cc. 150   | cc. 150   | cc. 150   | cc. 150   | cc. 150   | cc. 150   | cc. 150   |
| 1-Hydroxy-2-naphthoyl cyclohexylamide            | g. 2      | g. 2      | g. 2      | g. 2      | g. 2      | g. 2      | g. 2      |
| 2-Amino-5-diethylamino toluene                   | g. 2      | g. 2      | g. 2      | g. 2      | g. 2      | g. 2      | g. 2      |
| Water to make                                    | cc. 1,000 | cc. 1,000 | cc. 1,000 | cc. 1,000 | cc. 1,000 | cc. 1,000 | cc. 1,000 |
| Delay period in onset of scum in hours (approx.) | nil       | 2         | 2         | 12        | 12        | 12        | 48        |

When, in Developer G the tetronimide was replaced by 4-phenyl-2-oxytetronic acid (Example H), a similar delay in scum formation for 48 hours was obtained.

The pH of the developer was in all cases approximately 10.50. It will be seen that while hydroxylamine alone is ineffective at this pH, and both ascorbic acid and a typical tetronic compound afford only limited protection against scum formation, the combination of the two (developers D, E, F, G and H) shows a very much enhanced protective effect.

What I claim is:

1. A photographic developing composition for use in colour developing a developable silver salt image in a photographic element which comprises an aqueous alkaline solution of an aromatic primary amino developing agent, a colour coupler which is capable of combining with the oxidation products of such developer to form a dye, a compound selected from the class consisting of hydroxylamine and its salts and a compound selected from the class consisting of ascorbic acid and tetronic compounds of the formula:



where R is selected from the class consisting of phenyl and naphthyl groups, and phenyl and naphthyl groups containing alkyl, aralkyl, aryl, sulphonic acid and halogen substituents, and X is selected from the class consisting of the oxygen atom and the imino group.

2. A photographic developing composition for use in colour developing a developable silver salt image in a

photographic element which comprises an aqueous alkaline solution of an aromatic primary amino developing agent, a colour coupler which is capable of combining with the oxidation products of such developer to form a dye, a compound selected from the class consisting of hydroxylamine and its salts in a concentration of 0.5 to 1.5 g./litre and a compound selected from the class consisting of ascorbic acid and tetronic compounds of the formula:



where R is selected from the class consisting of phenyl and naphthyl groups, and phenyl and naphthyl groups containing alkyl, aralkyl, aryl, sulphonic acid and halogen substituents, and X is selected from the class consisting of the oxygen atom and the imino group in a concentration of 0.1 to 0.5 g./litre.

3. A photographic developing composition for use in colour developing a developable silver salt image in a photographic element which comprises an aqueous solution of pH 9 to 11.25 of an aromatic primary amino

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15

25

10

5

20

15</p

colour developing a developable silver salt image in a photographic element which comprises an aqueous solution of pH 9 to 11.25 of an aromatic primary amino developing agent, a colour coupler which is capable of combining with the oxidation products of such developing agent to form a dye, alkali carbonate, hydroxylamine in a concentration of 0.5 to 1.5 g./litre, and 4-phenyl-2-oxytetronimide in a concentration of 0.1 to 0.5 g./litre.

8. A photographic developing composition for use in colour developing a developable silver salt image in a photographic element which comprises an aqueous solution of pH 9 to 11.25 of an aromatic primary amino developing agent, a colour coupler which is capable of combining with the oxidation products of such developing agent to form a dye, alkali carbonate, hydroxylamine in a concentration of 0.5 to 1.5 g./litre, and 4-phenyl-2-oxytetronimide in a concentration of 0.1 to 0.5 g./litre.

9. A photographic developing composition for use in colour developing a developable silver salt image in a photographic element, which comprises an aqueous solution of pH 9 to 11.25 of an aromatic primary amino developing agent, a colour coupler which is capable of combining with the oxidation products of such developing agent to form a dye, tribasic sodium phosphate, dibasic sodium phosphate, hydroxylamine in a concentration of 0.5 to 1.5 g./litre, and ascorbic acid in a concentration of 0.1 to 0.5 g./litre.

10. A photographic developing composition for use in colour developing a developable silver salt image in a

photographic element which comprises an aqueous solution of pH 9 to 11.25 of an aromatic primary amino developing agent, a colour coupler which is capable of combining with the oxidation products of such developing agent to form a dye, tribasic sodium phosphate, dibasic sodium phosphate, hydroxylamine in a concentration of 0.5 to 1.5 g./litre, and 4-phenyl-2-oxytetronimide in a concentration of 0.1 to 0.5 g./litre.

11. A photographic developing composition for use in colour developing a developable silver salt image in a photographic element which comprises an aqueous solution of pH 9 to 11.25 of an aromatic primary amino developing agent, a colour coupler which is capable of combining with the oxidation products of such developing agent to form a dye, tribasic sodium phosphate, dibasic sodium phosphate, hydroxylamine in a concentration of 0.5 to 1.5 g./litre, and 4-phenyl-2-oxytetronimide in a concentration of 0.1 to 0.5 g./litre.

References Cited in the file of this patent

UNITED STATES PATENTS

|           |                     |               |
|-----------|---------------------|---------------|
| 2,286,662 | Weyde et al. -----  | June 16, 1942 |
| 2,401,713 | Vittum et al. ----- | June 4, 1946  |
| 2,656,272 | Gunther -----       | Oct. 20, 1953 |

FOREIGN PATENTS

|         |                     |               |
|---------|---------------------|---------------|
| 751,304 | Great Britain ----- | June 27, 1956 |
|---------|---------------------|---------------|